

# United States Patent [19]

Wollenberg

[11] Patent Number: 4,755,312

[45] Date of Patent: Jul. 5, 1988

[54] CARBONATE TREATED DISPERSANTS

[75] Inventor: Robert H. Wollenberg, San Rafael, Calif.

[73] Assignee: Chevron Research Company, San Francisco, Calif.

[21] Appl. No.: 910,107

[22] Filed: Sep. 19, 1986

Related U.S. Application Data

[62] Division of Ser. No. 834,972, Feb. 28, 1986, Pat. No. 4,729,842, which is a division of Ser. No. 673,963, Nov. 21, 1984, Pat. No. 4,585,566.

[51] Int. Cl.<sup>4</sup> ..... C10M 133/16

[52] U.S. Cl. ..... 252/51.5 A; 252/51.5 R; 548/545; 549/228; 549/229

[58] Field of Search ..... 252/51.5 A, 51.5 R; 548/545; 549/228, 229

[56] References Cited

U.S. PATENT DOCUMENTS

|           |         |                |           |
|-----------|---------|----------------|-----------|
| 2,802,022 | 8/1957  | Groszos et al. | 260/471   |
| 2,844,449 | 7/1958  | Dille et al.   | 44/70     |
| 2,921,955 | 1/1960  | Newman et al.  | 260/463   |
| 2,991,162 | 7/1961  | Malec          | 44/58     |
| 3,216,936 | 11/1965 | Le Suér        | 252/32.7  |
| 3,367,943 | 2/1968  | Miller et al.  | 260/326.3 |

|           |         |                   |            |
|-----------|---------|-------------------|------------|
| 3,373,111 | 3/1968  | Le Suer et al.    | 252/51.5   |
| 3,652,240 | 3/1972  | Dorn et al.       | 44/66      |
| 4,234,435 | 11/1980 | Meinhardt et al.  | 252/51.5 A |
| 4,322,305 | 3/1982  | Lewis             | 252/51.5 A |
| 4,410,437 | 10/1983 | Erdman            | 252/47.5   |
| 4,460,381 | 7/1984  | Karol et al.      | 44/63      |
| 4,482,464 | 11/1984 | Karol et al.      | 252/51.5 A |
| 4,490,154 | 12/1984 | Sung et al.       | 44/70      |
| 4,501,597 | 2/1985  | Karol et al.      | 44/63      |
| 4,584,117 | 4/1986  | Wollenberg        | 252/51.5 A |
| 4,585,566 | 4/1986  | Wollenberg        | 252/51.5 A |
| 4,612,132 | 9/1986  | Wollenberg et al. | 252/51.5 A |

FOREIGN PATENT DOCUMENTS

689705 4/1953 United Kingdom .

Primary Examiner—Jacqueline V. Howard  
Attorney, Agent, or Firm—S. R. LaPaglia; R. C. Gaffney; G. F. Swiss

[57]

ABSTRACT

Disclosed are additives which are useful as dispersants in marine crankcase oils and hydraulic oils, lubricating oils. In particular, disclosed are nitrogen-containing lubricating oil dispersants having at least one primary or secondary amino group which have been modified by treatment with a cyclic carbonate.

20 Claims, No Drawings

## CARBONATE TREATED DISPERSANTS

This is a division of application Ser. No. 834,972, filed Feb. 28, 1986, now U.S. Pat. No. 4,729,842, which in turn is a division of application Ser. No. 673,963, filed Nov. 21, 1984, now U.S. Pat. No. 4,585,566.

## FIELD OF THE INVENTION

Lubricating oil additives are prepared by reacting a dispersant composition containing at least one primary or secondary amino group with a cyclic carbonate.

## DESCRIPTION OF THE PRIOR ART

Most commercial lubricating oils now contain dispersant additives to help keep the engine clean by dispersing sludge and varnish-forming deposits in the oil. Many of these dispersant additives contain basic nitrogen as primary or secondary amino groups.

Primary and secondary amino groups of a succinimide dispersant have been previously modified by treatment with an alkylene oxide (see U.S. Pat. Nos. 3,373,111 and 3,367,943). U.S. Pat. No. 2,991,162 and U.S. Pat. No. 3,652,240 disclose motor fuel additives which have been modified by treatment with ethylene carbonate.

Likewise, my previously filed pending application, U.S. Ser. No. 632,777, teaches the preparation of modified alkenyl or alkyl succinimide by treatment with a cyclic carbonate. These modified succinimides are disclosed as possessing enhanced dispersancy over the unmodified succinimides.

## SUMMARY OF THE INVENTION

In addition to succinimides, it has now been found that the dispersant performance of other nitrogen-containing lubricating oil additives having at least one primary or secondary amino group is improved by reaction with a cyclic carbonate. Included among these additives are Mannich bases, borated Mannich bases, hydrocarbyl sulfonamides having at least one additional amino group, N-alkylaminophosphoramides, polyoxy-alkylene polyamines and amino-decorated hydrogen polymers. Accordingly, the present invention is directed to an improved lubricating oil dispersant additive prepared by the process comprising contacting at a temperature sufficient to cause a reaction a nitrogen-containing lubricating oil dispersant having at least one primary or secondary amino group with a cyclic carbonate.

As noted above, the modified dispersants of this invention possess improved dispersancy properties. Thus, another aspect of this invention is a lubricating oil composition comprising a major amount of an oil of lubricating viscosity and a dispersant effective amount of a modified dispersant of this invention.

## DETAILED DESCRIPTION OF THE INVENTION

The modified lubricating oil dispersants of this invention are prepared by reaction of a nitrogen-containing dispersant having at least one primary or secondary amino group with a cyclic carbonate. The reaction is conducted at a temperature sufficient to cause reaction of the cyclic carbonate with the primary or secondary amino group of the dispersant. In particular, reaction temperatures of from about 0° C. to about 250° C. are

preferred with temperatures of from about 100° C. to 200° C. being most preferred.

The reaction may be conducted neat - that is, both the dispersant and the carbonate are combined in the proper ratio, either alone or in the presence of a catalyst, such as an acidic, basic or Lewis acid catalyst, and then stirred at the reaction temperature. Examples of suitable catalysts include, for instance, boron trifluoride, alkane sulfonic acid, alkali or alkaline carbonate.

Alternatively, the reaction may be conducted in a diluent. For example, the reactants may be combined in a solvent such as toluene, xylene, oil or the like, and then stirred at the reaction temperature. After reaction completion, volatile components may be stripped off. When a diluent is employed, it is preferably inert to the reactants and products formed and is generally used in an amount sufficient to insure efficient stirring.

Water, which can be present in the dispersant, may be removed from the reaction system either before or during the course of the reaction via azeotroping or distillation. After reaction completion, the system can be stripped at elevated temperatures (100° C. to 250° C. and reduced pressure to remove any volatile components which may be present in the product.

Mole ratios of the cyclic carbonate to the basic amine nitrogen of the dispersant employed in the process of this invention are generally in the range of from about 0.2:1 to about 10:1, although preferably from about 0.5:1 to about 5:1 and most preferably 1:1 to 3:1.

The reaction is generally complete from within 0.5 to 10 hours.

## A. Carbonates

Cyclic carbonates employed in this invention react with a basic primary or secondary amine to form either a corresponding carbamate or a hydroxyalkylamine derivative. Suitable cyclic carbonates include:



60  
65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
340  
341  
342  
343  
344  
345  
346  
347  
348  
349  
350  
351  
352  
353  
354  
355  
356  
357  
358  
359  
360  
361  
362  
363  
364  
365  
366  
367  
368  
369  
370  
371  
372  
373  
374  
375  
376  
377  
378  
379  
380  
381  
382  
383  
384  
385  
386  
387  
388  
389  
390  
391  
392  
393  
394  
395  
396  
397  
398  
399  
400  
401  
402  
403  
404  
405  
406  
407  
408  
409  
410  
411  
412  
413  
414  
415  
416  
417  
418  
419  
420  
421  
422  
423  
424  
425  
426  
427  
428  
429  
430  
431  
432  
433  
434  
435  
436  
437  
438  
439  
440  
441  
442  
443  
444  
445  
446  
447  
448  
449  
450  
451  
452  
453  
454  
455  
456  
457  
458  
459  
460  
461  
462  
463  
464  
465  
466  
467  
468  
469  
470  
471  
472  
473  
474  
475  
476  
477  
478  
479  
480  
481  
482  
483  
484  
485  
486  
487  
488  
489  
490  
491  
492  
493  
494  
495  
496  
497  
498  
499  
500  
501  
502  
503  
504  
505  
506  
507  
508  
509  
510  
511  
512  
513  
514  
515  
516  
517  
518  
519  
520  
521  
522  
523  
524  
525  
526  
527  
528  
529  
530  
531  
532  
533  
534  
535  
536  
537  
538  
539  
540  
541  
542  
543  
544  
545  
546  
547  
548  
549  
550  
551  
552  
553  
554  
555  
556  
557  
558  
559  
560  
561  
562  
563  
564  
565  
566  
567  
568  
569  
570  
571  
572  
573  
574  
575  
576  
577  
578  
579  
580  
581  
582  
583  
584  
585  
586  
587  
588  
589  
590  
591  
592  
593  
594  
595  
596  
597  
598  
599  
600  
601  
602  
603  
604  
605  
606  
607  
608  
609  
610  
611  
612  
613  
614  
615  
616  
617  
618  
619  
620  
621  
622  
623  
624  
625  
626  
627  
628  
629  
630  
631  
632  
633  
634  
635  
636  
637  
638  
639  
640  
641  
642  
643  
644  
645  
646  
647  
648  
649  
650  
651  
652  
653  
654  
655  
656  
657  
658  
659  
660  
661  
662  
663  
664  
665  
666  
667  
668  
669  
670  
671  
672  
673  
674  
675  
676  
677  
678  
679  
680  
681  
682  
683  
684  
685  
686  
687  
688  
689  
690  
691  
692  
693  
694  
695  
696  
697  
698  
699  
700  
701  
702  
703  
704  
705  
706  
707  
708  
709  
710  
711  
712  
713  
714  
715  
716  
717  
718  
719  
720  
721  
722  
723  
724  
725  
726  
727  
728  
729  
730  
731  
732  
733  
734  
735  
736  
737  
738  
739  
740  
741  
742  
743  
744  
745  
746  
747  
748  
749  
750  
751  
752  
753  
754  
755  
756  
757  
758  
759  
760  
761  
762  
763  
764  
765  
766  
767  
768  
769  
770  
771  
772  
773  
774  
775  
776  
777  
778  
779  
780  
781  
782  
783  
784  
785  
786  
787  
788  
789  
790  
791  
792  
793  
794  
795  
796  
797  
798  
799  
800  
801  
802  
803  
804  
805  
806  
807  
808  
809  
8010  
8011  
8012  
8013  
8014  
8015  
8016  
8017  
8018  
8019  
8020  
8021  
8022  
8023  
8024  
8025  
8026  
8027  
8028  
8029  
8030  
8031  
8032  
8033  
8034  
8035  
8036  
8037  
8038  
8039  
8040  
8041  
8042  
8043  
8044  
8045  
8046  
8047  
8048  
8049  
8050  
8051  
8052  
8053  
8054  
8055  
8056  
8057  
8058  
8059  
8060  
8061  
8062  
8063  
8064  
8065  
8066  
8067  
8068  
8069  
8070  
8071  
8072  
8073  
8074  
8075  
8076  
8077  
8078  
8079  
8080  
8081  
8082  
8083  
8084  
8085  
8086  
8087  
8088  
8089  
8090  
8091  
8092  
8093  
8094  
8095  
8096  
8097  
8098  
8099  
80100  
80101  
80102  
80103  
80104  
80105  
80106  
80107  
80108  
80109  
80110  
80111  
80112  
80113  
80114  
80115  
80116  
80117  
80118  
80119  
80120  
80121  
80122  
80123  
80124  
80125  
80126  
80127  
80128  
80129  
80130  
80131  
80132  
80133  
80134  
80135  
80136  
80137  
80138  
80139  
80140  
80141  
80142  
80143  
80144  
80145  
80146  
80147  
80148  
80149  
80150  
80151  
80152  
80153  
80154  
80155  
80156  
80157  
80158  
80159  
80160  
80161  
80162  
80163  
80164  
80165  
80166  
80167  
80168  
80169  
80170  
80171  
80172  
80173  
80174  
80175  
80176  
80177  
80178  
80179  
80180  
80181  
80182  
80183  
80184  
80185  
80186  
80187  
80188  
80189  
80190  
80191  
80192  
80193  
80194  
80195  
80196  
80197  
80198  
80199  
80200  
80201  
80202  
80203  
80204  
80205  
80206  
80207  
80208  
80209  
80210  
80211  
80212  
80213  
80214  
80215  
80216  
80217  
80218  
80219  
80220  
80221  
80222  
80223  
80224  
80225  
80226  
80227  
80228  
80229  
80230  
80231  
80232  
80233  
80234  
80235  
80236  
80237  
80238  
80239  
80240  
80241  
80242  
80243  
80244  
80245  
80246  
80247  
80248  
80249  
80250  
80251  
80252  
80253  
80254  
80255  
80256  
80257  
80258  
80259  
80260  
80261  
80262  
80263  
80264  
80265  
80266  
80267  
80268  
80269  
80270  
80271  
80272  
80273  
80274  
80275  
80276  
80277  
80278  
80279  
80280  
80281  
80282  
80283  
80284  
80285  
80286  
80287  
80288  
80289  
80290  
80291  
80292  
80293  
80294  
80295  
80296  
80297  
80298  
80299  
80300  
80301  
80302  
80303  
80304  
80305  
80306  
80307  
80308  
80309  
80310  
80311  
80312  
80313  
80314  
80315  
80316  
80317  
80318  
80319  
80320  
80321  
80322  
80323  
80324  
80325  
80326  
80327  
80328  
80329  
80330  
80331  
80332  
80333  
80334  
80335  
80336  
80337  
80338  
80339  
80340  
80341  
80342  
80343  
80344  
80345  
80346  
80347  
80348  
80349  
80350  
80351  
80352  
80353  
80354  
80355  
80356  
80357  
80358  
80359  
80360  
80361  
80362  
80363  
80364  
80365  
80366  
80367  
80368  
80369  
80370  
80371  
80372  
80373  
80374  
80375  
80376  
80377  
80378  
80379  
80380  
80381  
80382  
80383  
80384  
80385  
80386  
80387  
80388  
80389  
80390  
80391  
80392  
80393  
80394  
80395  
80396  
80397  
80398  
80399  
80400  
80401  
80402  
80403  
80404  
80405  
80406  
80407  
80408  
80409  
80410  
80411  
80412  
80413  
80414  
80415  
80416  
80417  
80418  
80419  
80420  
80421  
80422  
80423  
80424  
80425  
80426  
80427  
80428  
80429  
80430  
80431  
80432  
80433  
80434  
80435  
80436  
80437  
80438  
80439  
80440  
80441  
80442  
80443  
80444  
80445  
80446  
80447  
80448  
80449  
80450  
80451  
80452  
80453  
80454  
80455  
80456  
80457  
80458  
80459  
80460  
80461  
80462  
80463  
80464  
80465  
80466  
80467  
80468  
80469  
80470  
80471  
80472  
80473  
80474  
80475  
80476  
80477  
80478  
80479  
80480  
80481  
80482  
80483  
80484  
80485  
80486  
80487  
80488  
80489  
80490  
80491  
80492  
80493  
80494  
80495  
80496  
80497  
80498  
80499  
80500  
80501  
80502  
80503  
80504  
80505  
80506  
80507  
80508  
80509  
80510  
80511  
80512  
80513  
80514  
80515  
80516  
80517  
80518  
80519  
80520  
80521  
80522  
80523  
80524  
80525  
80526  
80527  
80528  
80529  
80530  
80531  
80532  
80533  
80534  
80535  
80536  
80537  
80538  
80539  
80540  
80541  
80542  
80543  
80544  
80545  
80546  
80547  
80548  
80549  
80550  
80551  
80552  
80553  
80554  
80555  
80556  
80557  
80558  
80559  
80560  
80561  
80562  
80563  
80564  
80565  
80566  
80567  
80568  
80569  
80570  
80571  
80572  
80573  
80574  
80575  
80576  
80577  
80578  
80579  
80580  
80581  
80582  
80583  
80584  
80585  
80586  
80587  
80588  
80589  
80590  
80591  
80592  
80593  
80594  
80595  
80596  
80597  
80598  
80599  
80600  
80601  
80602  
80603  
80604  
80605  
80606  
80607  
80608  
80609  
80610  
80611  
80612  
80613  
80614  
80615  
80616  
80617  
80618  
80619  
80620  
80621  
80622  
80623  
80624  
80625  
80626  
80627  
80628  
80629  
80630  
80631  
80632  
80633  
80634  
80635  
80636  
80637  
80638  
80639  
80640  
80641  
80642  
80643  
80644  
80645  
80646  
80647  
80648  
80649  
80650  
80651  
80652  
80653  
80654  
80655  
80656  
80657  
80658  
80659  
80660  
80661  
80662  
80663  
80664  
80665  
80666  
80667  
80668  
80669  
80670  
80671  
80672  
80673  
80674  
80675  
80676  
80677  
80678  
80679  
80680  
80681  
80682  
80683  
80684  
80685  
80686  
80687  
80688  
80689  
80690  
80691  
80692  
80693  
80694  
80695  
80696  
80697  
80698  
80699  
80700  
80701  
80702  
80703  
80704  
80705  
80706  
80707  
80708  
80709  
80710  
80711  
80712  
80713  
80714  
80715  
80716  
80717  
80718  
80719  
80720  
80721  
80722  
80723  
80724  
80725  
80726  
80727  
80728  
80729  
80730  
80731  
80732  
80733  
80734  
80735  
80736  
80737  
80738  
80739  
80740  
80741  
80742  
80743  
80744  
80745  
80746  
80747  
80748  
80749  
80750  
80751  
80752  
80753  
80754  
80755  
80756  
80757  
80758  
80759  
80760  
8

Preferred cyclic carbonates for use in this invention are those of formula 1 above. Preferred R<sub>1</sub>, R<sub>2</sub>, R<sub>3</sub>, R<sub>4</sub>, R<sub>5</sub> and R<sub>6</sub> are either hydrogen or methyl. Most preferably R<sub>1</sub>, R<sub>2</sub>, R<sub>3</sub>, R<sub>4</sub>, R<sub>5</sub> and R<sub>6</sub> are hydrogen, when n is one. R<sub>6</sub> is most preferably hydrogen or methyl while R<sub>1</sub>, R<sub>2</sub>, and R<sub>5</sub> are hydrogen when n is zero.

The following are examples of suitable cyclic carbonates for use in this invention: 1,3-dioxolan-2-one(ethylene carbonate); 4-methyl-1,3-dioxolan-2-one(propylene carbonate); 4-hydroxymethyl-1,3-dioxolan-2-one; 4,5-dimethyl-1,3-dioxolan-2-one; 4-ethyl-1,3-dioxolan-2-one; 4,4-dimethyl-1,3-dioxolan-2-one; 4-methyl-5-ethyl-1,3-dioxolan-2-one; 4,5-diethyl-1,3-dioxolan-2-one; 4,4-diethyl-1,3-dioxolan-2-one; 1,3-dioxan-2-one; 4,4-dimethyl-1,3-dioxan-2-one; 5,5-dimethyl-1,3-dioxan-2-one; 5,5-dihydroxymethyl-1,3-dioxan-2-one; 5-methyl-1,3-dioxan-2-one; 4-methyl-1,3-dioxan-2-one; 5-hydroxy-1,3-dioxan-2-one; 5,5-diethyl-1,3-dioxan-2-one; 5-methyl-5-propyl-1,3-dioxan-2-one; 4,6-dimethyl-1,3-dioxan-2-one; 4,4,6-trimethyl-1,3-dioxan-2-one and spiro[1,3-oxa-2-cyclohexanone-5,5'-1',3'-oxa-2'-cyclohexanone].

Several of these cyclic carbonates are commercially available such as 1,3-dioxolan-2-one or 4-methyl-1,3-dioxolan-2-one. Cyclic carbonates may be readily prepared by known reactions. For example, reaction of phosgene with a suitable alpha alkane diol or an alkan-1,3-diol yields a carbonate for use within the scope of this invention (see U.S. Pat. No. 4,115,206).

Likewise, the cyclic carbonates useful for this invention may be prepared by transesterification of a suitable alpha alkane diol or an alkan-1,3-diol with, e.g., diethyl carbonate under transesterification conditions. See, for instance, U.S. Pat. Nos. 4,384,115 and 4,423,205 which are incorporated herein by reference for their teaching of the preparation of cyclic carbonates.

As used herein, the term "alpha alkane diol" means an alkane group having two hydroxyl substituents wherein the hydroxyl substituents are on adjacent carbons to each other. Examples of alpha alkane diols include 1,2-propanediol, 2,3-butanediol and the like.

The term "alkan-1,3-diol" means an alkane group having two hydroxy substituents wherein the hydroxyl substituents are beta substituted. That is, there is a methylene or a substituted methylene moiety between the hydroxyl substituted carbons. Examples of alkan-1,3-diols include propan-1,3-diol, pentan-2,4-diol and the like.

As used herein, the term "spiro[1,3-oxa-2-cyclohexanone-5,5'-1',3'-oxa-2'-cyclohexanone" means the group



As used herein, the term "molar charge of cyclic carbonate to the basic nitrogen of the dispersant" means that the molar charge of cyclic carbonate employed in the reaction is based upon the theoretical number of

basic nitrogens (i.e., nitrogens titratable by a strong acid) contained in the dispersant. Thus, when 1 equivalent of triethylene tetraamine (TETA) is reacted with an equivalent of hydrocarbyl carboxylic acid, the resulting amide will theoretically contain 3 basic nitrogens. Accordingly, a molar charge of 1 would require that a mole of cyclic carbonate be added for each basic nitrogen or in this case 3 moles of cyclic carbonate for each mole of amide prepared from TETA.

The alpha alkane diols, used to prepare the 1,3-dioxolan-2-ones employed in this invention, are either commercially available or may be prepared from the corresponding olefin by methods known in the art. For example, the olefin may first react with a peracid, such as peroxyacetic acid or hydrogen peroxide plus formic acid to form the corresponding epoxide which is readily hydrolyzed under acid or base catalysis to the alpha alkane diol. In another process, the olefin is first halogenated to a dihalo derivative and subsequently hydrolyzed to an alpha alkane diol by reaction first with sodium acetate and then with sodium hydroxide. The olefins so employed are known in the art.

The alkan-1,3-diols, used to prepare the 1,3-dioxan-2-ones employed in this invention, are either commercially available or may be prepared by standard techniques, e.g., derivatizing malonic acid.

4-Hydroxymethyl 1,3-dioxolan-2-one derivatives and 5-hydroxy-1,3-dioxan-2-one derivatives may be prepared by employing glycerol or substituted glycerol in the process of U.S. Pat. No. 4,115,206. The mixture so prepared may be separated, if desired, by conventional techniques. Preferably the mixture is used as is.

5,5-Dihydroxymethyl-1,3-dioxan-2-one may be prepared by reacting an equivalent of pentaerythritol with an equivalent of either phosgene or diethylcarbonate (or the like) under transesterification conditions.

Spiro[1,3-oxa-2-cyclohexanone-5,5'-1',3'-oxa-2'-cyclohexanone] may be prepared by reacting an equivalent of pentaerythritol with two equivalents of either phosgene or diethylcarbonate (or the like) under transesterification conditions.

#### B. Nitrogen-Containing Dispersants

The dispersants whose performance is improved by the process of this invention must contain at least one basic nitrogen and have at least one >NH group. The essence of this invention resides in the surprising discovery that treating the lubricating oil dispersant with a cyclic carbonate improves its dispersant properties. The dispersants include Mannich bases, borated Mannich bases, hydrocarbyl sulfonamides having at least one additional amino group, N-alkylaminophosphoramides, polyoxyalkylene polyamines, and amino-decorated hydrocarbon polymers useful as dispersant-viscosity index improvers.

The Mannich bases used for preparing the additives of this invention are also well known. Representative types of Mannich bases are described in U.S. Pat. Nos. 3,741,896, 3,539,633 and 3,649,229, the disclosures of which are hereby incorporated by reference. In general, the Mannich bases are prepared by reacting an alkylphenol, formaldehyde, and a mono- or polyamine. The Mannich base may be borated by reacting with, e.g., a boron halide, boric acid, or an ester of boric acid. Preferred amines for use in forming the Mannich base are methylamine and ethylenamines such as ethylenediamine, diethylenetriamine, and triethylenetetraamine.

The hydrocarbyl sulfonamides for use in preparing the additives of this invention are described in U.S. Pat. No. 4,122,266, the disclosure of which is hereby incorporated by reference. The sulfonamides are preferably prepared from a hydrocarbyl sulfonyl chloride and an amine. Particularly preferred are the reaction products of polyisobutylene sulfonyl chloride containing 50 to 300 carbon atoms and an ethylene amine such as diethylenetriamine, triethylenetetraamine, and tetraethylenepentamine.

Amino-decorated hydrocarbon polymers useful as dispersant viscosity index improvers are usually prepared by treating a hydrocarbon polymer having viscosity index improving characteristics, such as an ethylene-propylene copolymer or terpolymer, either chemically or mechanically to generate active sites and then reacting with an amine or polyamine. Typical products are prepared by oxidizing the copolymer or terpolymer and reacting with an amine as shown in U.S. Pat. No. 3,769,216 or with an amine an aldehyde as shown in U.S. Pat. No. 3,872,019, the disclosure of which are hereby incorporated by reference.

Similarly, other primary or secondary amine-substituted polymers used as viscosity-index improvers may be used as starting materials for the additives of the invention. Such polymers include amine-grafted acrylic polymers and copolymers and copolymers wherein one monomer contains at least one amino group. Typical compositions are described in British Pat. No. 1,488,382, U.S. Pat. Nos. 4,089,794 and 4,025,452, the disclosures of which are incorporated herein by reference.

The polyoxyalkylene polyamine additives consists of three parts or moieties. The first is the polyether or polyoxyalkylene moiety, which may or may not be hydrocarbyl terminated or "capped". The polyether moiety is bound through the second moiety, a connecting group or linkage to the nitrogen atom of the third moiety, the amine.

#### Polyoxyalkylene Moeity

The polyoxyalkylene moiety is ordinarily comprised of polyoxyalkylene polymers containing at least one oxyalkylene unit, preferably 1 to 30 units, and more preferably 5 to 30 units, and most preferably 10 to about 25 oxyalkylene units. When polymerized in the polymerization reaction, a single type of alkylene oxide may be employed. Copolymers, however, are equally satisfactory and random copolymers are readily prepared. Blocked copolymers of oxyalkylene units also provide satisfactory polyoxyalkylene polymers for the practice of the present invention.

The polyoxyalkylene moiety may also be terminated or "capped" by a hydrocarbyl terminating group. This terminating group may be comprised of an alkyl group of from 5 to about 30 carbon atoms, an aryl group of from 6 to about 30 carbon atoms, an alkaryl group of from 7 to about 30 carbon atoms, an aralkyl group of from 7 to about 30 carbon atoms, or a methylol-substituted alkyl group of from 5 to about 10 carbon atoms.

The polyoxyalkylene moiety may ordinarily be prepared in a variety of ways, the most common for the practice of the present invention being by the reaction of an appropriate lower alkylene oxide containing from 2 to 4 carbon atoms with an appropriate initiator; for example, chlorohydrin or an alkyl phenol. In a preferred embodiment, ethylene chlorohydrin is used. Copolymers may be readily prepared by contacting the

initiator compound with a mixture of alkylene oxides, while the blocked copolymers may be prepared by reacting the initiator first with one alkylene oxide and then another in any order or repetitively under polymerization conditions.

As an example, the polyoxyalkylene moiety derived from an alkyl phenol initiated polymerization detailed above is prepared as an alcohol containing a terminal hydroxyl group. The polyether moiety is then attached through the appropriate connecting group to the polyamine moiety by a variety of ways, one of which includes reacting the hydroxyl group of the polyoxyalkylene unit with phosgene to form a polyoxyalkylene chloroformate and then reacting the polyoxyalkylene chloroformate with an amine. Alternatively, the hydroxyl group may be reacted with epichlorohydrin to give a methylol-substituted ethyl chloride end group. The resulting polyoxyalkylene alkyl chloride is then reacted with an amine or polyamine to produce the composition to be quaternized, resulting in the composition of the present invention.

#### The Connecting Group

The connecting group joining the polyoxyalkylene moiety with the amine moiety may be any relatively small diradical containing at least one carbon, oxygen, sulfur and/or nitrogen atom, and usually containing up to 12 carbon atoms. The connecting group which results and is used in the present composition is ordinarily a function of the method by which the compositions are formed and/or by which the components of the polyoxyalkylene moiety and the polyamine moiety are joined together. Appropriate connecting groups include:



where Z and Z' independently = H, or an alkyl group of from 1 to 2 carbon atoms.

### The Amine Moiety

The amine moiety of the polyoxyalkylene polyamine is derived from ammonia or, more preferably, from a polyamine having from about 2 to about 12 amine nitrogen atoms and from about 2 to about 40 carbon atoms. The polyamine preferably has a carbon to nitrogen ratio of from about 1:1 to about 10:1. The polyamine may be substituted with a substituent group selected from (A) hydrogen; (B) hydrocarbyl groups from about 1 to about 10 carbon atoms; (C) acyl groups from about 2 to about 10 carbon atoms; and (D) monoketo, monocyano, lower alkyl and lower alkoxy derivatives of (B), (C). "Lower", as used in lower alkyl and lower alkoxy, means a group containing about 1 to 6 carbon atoms. "Hydrocarbyl" denotes an organic radical composed of carbon and hydrogen which may be aliphatic, alicyclic, aromatic or combinations thereof, e.g., aralkyl. The substituted polyamines of the present invention are generally, but not necessarily, N-substituted polyamines. The acyl groups falling within the definition of the aforementioned (C) substituents are such as propionyl, acetyl, etc. The more preferred substituents are hydrogen, C<sub>1</sub> to C<sub>6</sub> alkyls, and C<sub>1</sub>-C<sub>6</sub> hydroxyalkyls.

The more preferred polyamines finding use within the scope of the present invention are polyalkylene polyamines, including alkylene diamine and substituted polyamines, e.g., alkyl and hydroxyalkyl-substituted polyalkylene polyamines. Preferably the alkylene groups contain from 2 to 6 carbon atoms, there being preferably from 2 to 3 carbon atoms between the nitrogen atoms. Such groups are exemplified by ethylenamines and include ethylene diamine, diethylene triamine, di(trimethylene) triamine, dipropyleneetriamine, triethylenetetramine, etc. Such amines encompass isomers which are the branched-chain polyamines and the previously mentioned substituted polyamines, including hydroxy and hydrocarbyl-substituted polyamines. Among the polyalkylene polyamines, those containing 2 to 12 amine nitrogen atoms and 2 to 24 carbon atoms, are especially preferred and the  $C_2$  to  $C_3$  alkylene polyamines are most preferred, in particular, the lower polyalkylene polyamines, e.g., ethylene diamine, tetraethylenepentamine, etc.

In many instances a single compound will not be used as reactant in the preparation of the compositions of this invention, in particular the polyamine component. That is, mixtures will be used in which one or two compounds will predominate with the average composition indicated.

A generalized, preferred formula for the polyoxayalkylene polyamines finding utility in this invention is as follows:



wherein

R=an alkyl group of 5 to 30 carbon atoms, aryl group of 6 to 30 carbon atoms, alkaryl group of 7 to 30 carbon atoms, aralkyl group of 7 to 30 carbon atoms, or methylol-substituted alkyl group of 5 to 30 carbon atoms;

$R^i$  and  $R^{ii}$  independently = hydrogen, methyl or ethyl;  
 $n = 1$  to 30, preferably 10 to 25;  
 $X$  = the connecting group as defined above:



where  $X=1$  to  $5$ .

### C. Modified Dispersant Complexes

10 Cyclic carbonates of Formula I are used to illustrate the reaction of the carbonate with a nitrogencontaining dispersant. It is to be understood that the other cyclic carbonates employed in this invention react similarly. Cyclic carbonates react with the primary and secondary amines of a dispersant to form two types of compounds. In the first instance, strong bases, including unhindered amines such as primary amines and some secondary amines, react with an equivalent of cyclic carbonate to produce a carbamic ester as shown in reaction (1) below:



35 wherein  $R_1$ ,  $R_2$ ,  $R_3$ ,  $R_4$ ,  $R_5$ ,  $R_6$  and  $n$  are as defined above and  $R_9$  is the remainder of a dispersant. In this reaction, the amine nitrogen has been rendered nonbasic by formation of the carbamate,  $V$ .

40 In the second instance, hindered bases, such as hindered secondary amines, may react with an equivalent of the same cyclic carbonate to form a hydroxyalkyleneamine linkage with the concomitant elimination of  $\text{CO}_2$  as shown below in reaction (2):



60 wherein  $R_1$ ,  $R_2$ ,  $R_3$ ,  $R_4$ ,  $R_5$ ,  $R_6$ ,  $R_9$  and  $n$  are as defined above and  $R_{10}$  is an alkyl or alkylene linking group which hinders the amine. Unlike the carbamate products of reaction (1), the hydroxyalkyleneamine products 65 of reaction (2) retain their basicity. These hydroxyalkyleneamine derivatives, VII, (when  $n=0$ ) are believed to be similar to those which are produced by the addition of a substituted ethylene oxide of the formula:



wherein R<sub>1</sub>, R<sub>2</sub>, R<sub>5</sub> and R<sub>6</sub> are as defined above. (See for instance U.S. Pat. Nos. 3,367,943 and 3,377,111).

In theory, if only primary and secondary amines are employed a determination of whether the carbonate addition follows reaction (1) or reaction (2) could be made by monitoring the AV (alkalinity value or alkalinity number - refers to the amount of base as milligrams of KOH in 1 gram of a sample) of the product. Accordingly, if the reaction proceeded entirely via reaction (1) above, a reaction product prepared by reacting an equivalent of carbonate for each basic nitrogen should yield an AV of zero. That is to say that all the basic amines in the polyamine moiety have been converted to nonbasic carbamates.

However, alkylene polyamines such as triethylene tetraamine and tetraethylene pentamine, contain tertiary amines (piperazines, etc.) which may account for as much as 30% of the basic nitrogen content. Although Applicant does not want to be limited to any theory, it is believed that these tertiary amines, although basic, are not reactive with the carbonate. Accordingly, even if the reaction proceeded entirely by reaction (1) above, an AV of approximately 30% of the original AV may be retained in the final product of such a polyamine. Nevertheless, a large drop in the AV of the product is significant evidence that a substantial portion of the reaction product contains carbamic esters.

In fact, the addition of the first molar charge of ethylene carbonate results in an appreciable lowering of the AV of the product.

The addition of a second molar charge of ethylene carbonate in these reactions does not result in appreciably further lowering of the AV. This suggests that the additional carbonate either reacts via reaction (2) above to form hydroxylalkyleneamine groups or are reacting with the hydroxyl group of the carbamate as shown in reaction 3(a) below:



wherein R<sub>1</sub>, R<sub>2</sub>, R<sub>3</sub>, R<sub>4</sub>, R<sub>5</sub>, R<sub>6</sub>, R<sub>9</sub> and n are as defined above.

The process of reaction 3(a) allows for additional carbonate to add to the hydroxyl group of product IX as shown in reaction 3(b) below:



wherein R<sub>1</sub>, R<sub>2</sub>, R<sub>3</sub>, R<sub>4</sub>, R<sub>5</sub>, R<sub>6</sub> and R<sub>10</sub> are as defined above. As is apparent from the above reaction, the poly(oxalkylene) portion of the carbamate can be repeated several times simply by addition of more carbonate.

Likewise, additional equivalents of carbonate could equally add to the hydroxyl group of the hydroxylalkyleneamine derivative, VII, of reaction (2) as shown in reaction (4) below:



wherein R<sub>1</sub>, R<sub>2</sub>, R<sub>3</sub>, R<sub>4</sub>, R<sub>5</sub>, R<sub>9</sub> and R<sub>10</sub> are as defined above. Repeating the process of reaction (4) above by the addition of increasing amounts of carbonate produces a hydroxylalkylenepoly(oxalkylene)amine derivative of Formula XII below:



wherein R<sub>1</sub>, R<sub>2</sub>, R<sub>3</sub>, R<sub>4</sub>, R<sub>8</sub>, R<sub>9</sub>, R<sub>10</sub> and n are as defined above and y is an integer from 3 to 10.

It is also contemplated that reactions (3) and (4) above may also produce acyclic carbonate linkages with the terminal hydroxyl group. Likewise, if R<sub>9</sub> (or R<sub>10</sub>) is hydrogen, then an additional hydroxylalkylene could add to the amino group.

Accordingly, it is expected that the reaction of a cyclic carbonate with a nitrogen-containing dispersant will yield a mixture of products. When the molar charge of the cyclic carbonate to the basic nitrogen of the dispersant is about 1 or less, it is anticipated that a large portion of the primary and secondary amines of the dispersant will have been converted to carbamic esters with some hydroxylalkyleneamine derivatives also being formed. As the molar charge is raised above 1, poly(oxalkylene) polymers of the carbamic esters and the

hydroxylalkyleneamine derivatives are expected.

It is expected that use of the spiro[1,3-oxa-2-cyclohexanone-5,5'-1',3'-oxa-2'-cyclohexanone] will yield materials which would be both internally cyclized and cross-linking between two dispersant molecules.

In some instances, it may be desirable to increase the proportion of carbamic esters formed in these reactions. This may be accomplished by employing a polyamine with a large percentage of primary amine. Another method may be to employ alkyl-substituted (i.e., one or more of R<sub>1</sub>, R<sub>2</sub>, R<sub>3</sub>, R<sub>4</sub>, R<sub>5</sub>, or R<sub>6</sub> is alkyl) or hydroxyl-substituted carbonates.

The modified dispersant of this invention can be reacted with boric acid or a similar boron compound to form borated dispersants having utility within the scope of this invention. In addition to boric acid (boron acid), examples of suitable boron compounds include boron oxides, boron halides and esters of boric acid. Generally from about 0.1 equivalents to 10 equivalents of boron compound to the modified dispersant may be employed.

The modified dispersants of this invention are useful as detergent and dispersant additives when employed in lubricating oils. When employed in this manner, the modified dispersant additive is usually present in from 0.2 to 10 percent by weight to the total composition and preferably at about 0.5 to 5 percent by weight. The lubricating oil used with the additive compositions of this invention may be mineral oil or synthetic oils of lubricating viscosity and preferably suitable for use in the crankcase of an internal combustion engine. Crankcase lubricating oils ordinarily have a viscosity of about 1300 CSt 0° F. to 22.7 CSt at 210° F. (99° C.). The lubricating oils may be derived from synthetic or natural sources. Mineral oil for use as the base oil in this invention includes paraffinic, naphthenic and other oils that are ordinarily used in lubricating oil compositions. Synthetic oils include both hydrocarbon synthetic oils and synthetic esters. Useful synthetic hydrocarbon oils include liquid polymers of alpha olefins having the proper viscosity. Especially useful are the hydrogenated liquid oligomers of C<sub>6</sub> to C<sub>12</sub> alpha olefins such as 1-decene trimer. Likewise, alkyl benzenes of proper viscosity such as didodecyl benzene, can be used. Useful synthetic esters include the esters of both monocarboxylic acid and polycarboxylic acids as well as monohydroxy alkanols and polyols. Typical examples are didodecyl adipate, pentaerythritol tetracaprate, di-2-ethylhexyl adipate, dilaurylsebacate and the like. Complex esters prepared from mixtures of mono and dicarboxylic acid and mono and dihydroxy alkanols can also be used.

Blends of hydrocarbon oils with synthetic oils are also useful. For example, blends of 10 to 25 weight percent hydrogenated 1-decene trimer with 75 to 90 weight percent 150 SUS (100° F.) mineral oil gives an excellent lubricating oil base.

Additive concentrates are also included within the scope of this invention. The concentrates of this invention usually include from about 90 to 10 weight percent of an oil of lubricating viscosity and from about 10 to 90 weight percent of the complex additive of this invention. Typically, the concentrates contain sufficient diluent to make them easy to handle during shipping and storage. Suitable diluents for the concentrates include any inert diluent, preferably an oil of lubricating viscosity, so that the concentrate may be readily mixed with lubricating oils to prepare lubricating oil compositions. Suitable lubricating oils which can be used as diluents typically have viscosities in the range from about 35 to about 500 Saybolt Universal Seconds (SUS) at 100° F. (38° C.), although an oil of lubricating viscosity may be used.

Other additives which may be present in the formulation include rust inhibitors, foam inhibitors, corrosion inhibitors, metal deactivators, pour point depressants, antioxidants, and a variety of other well-known additives.

It is also contemplated the modified dispersants of this invention may be employed as dispersants and detergents in hydraulic fluids, marine crankcase lubricants

and the like. When so employed, the modified dispersant is added at from about 0.1 to 10 percent by weight to the oil. Preferably, at from 0.5 to 5 weight percent.

The following examples are offered to specifically illustrate this invention. These examples and illustrations are not to be construed in any way as limiting the scope of this invention.

## EXAMPLES

### EXAMPLE 1

To a 500 ml reaction flask was charged 100 g of a hydrocarbyl amine dispersant, prepared from polyisobutylene chloride (where the polyisobutylene group has a number average weight of 1325) and ethylene diamine, containing about 50% diluent oil, and having an alkalinity value (AV)=41.6 mg KOH/g. 3.27 g Ethylene carbonate were added and the reaction mixture heated to 150° C. under N<sub>2</sub> and stirred for 4 hours. The mixture was then cooled, diluted with 200 ml 350° F. thinners, and stripped to 175° C. and 5 mm Hg. Recovered 102.1 g product having an AV=19.7 and containing 0.99% N.

### EXAMPLE 2

To a 500 ml reaction flask was charged 100 g of the hydrocarbyl amine dispersant described in Example 1 and 13.08 g ethylene carbonate. The reaction mixture was heated to 150° C. under N<sub>2</sub> and stirred for 4 hours. The mixture was then cooled, diluted with 200 ml 350° F. thinners, and stripped to 175° C. and 5 mm Hg. Recovered 112.9 g product having an AV=12.8 and containing 0.88% N.

### EXAMPLE 3

To a 500 ml reaction flask was charged 100 g of the hydrocarbyl amine dispersant of Example 1 and 7.44 g propylene carbonate. The reaction mixture was heated to 150° C. under N<sub>2</sub> and stirred for 4 hours. The mixture was then cooled, diluted with 200 ml 350° F. thinners, and stripped to 157° C. and 10 mm Hg. Recovered 106.6 g product having an AV=17.2 and containing 0.94% N.

### EXAMPLE 4

To a 500 ml reaction flask was charged 100 g of an amide detergent composition prepared from an aliphatic carboxylic acid of approximately 280 molecular weight and tetraethylenepentamine (where the ratio of carboxylic acid to polyamine is about 3 to 1 and having an AV=102). The amide was heated to 170° C. under N<sub>2</sub> and 16.5 g ethylene carbonate was added. The reaction mixture was then stirred at 170° C. for 4 hours. Recovered 112 g product having an AV=70.9 and containing 5.89% N.

### EXAMPLE 5

To a 500 ml reaction flask was charged 100 g of a poly(oxyalkylene) amino carbamate prepared by reacting a hydrocarbyl-capped poly(butylene oxide) chloroformate of approximately 1400 molecular weight with ethylene diamine and having an AV=10.9. The amine was heated to 170° C. under N<sub>2</sub> and 1.7 g ethylene carbonate added. The reaction mixture was then stirred at 170° C. for 4 hours. Recovered 101.3 g product having an AV=2.5 and containing 0.66% N.

## EXAMPLE 6

To a 500 ml reaction flask was charged 100 g of an amine-functionalized ethylene-propylene rubber of 5 30,000-200,000 MW in 89 g of lubricating diluent oil. The polymer was heated to 170° C. under N<sub>2</sub> and 0.1 g 10 ethylene carbonate added. The reaction mixture was stirred at 170° C. for 4 hours. Recovered 99.2 g product containing 131 ppm N.

## EXAMPLE 7

To a 500 ml reaction flask was charged 100 g of 15 Amoco 9050 (1.2% N; a Mannich dispersant prepared by reacting a polyisobutylene-substituted phenol with formaldehyde and a polyamine and having an AV=28.9). The Mannich dispersant was heated to 170° C. under N<sub>2</sub> and 14.0 g ethylene carbonate added. The 20 reaction mixture was stirred at 170° C. for 4 hours. Recovered 106.4 g product having an AV=20.7 and containing 1.07% N.

What is claimed is:

1. A product prepared by the process which comprises reacting at a temperature sufficient to cause reaction an amino-decorated hydrocarbon polymer having at least one primary or secondary amine group with a cyclic carbonate and wherein the molar charge of cyclic carbonate to the basic nitrogen of the amino-decorated hydrocarbon polymer is from about 0.2:1 to about 10:1.
2. A product prepared as in the process of claim 1 35 wherein the cyclic carbonate is selected from the group consisting of



- 40 11. A lubricating oil composition comprising an oil of lubricating viscosity and from 0.2 to 10 percent by weight of a product as defined in claim 3.
12. A lubricating oil composition comprising an oil of lubricating viscosity and from 0.2 to 10 percent by weight of a product as defined in claim 4.
13. A lubricating oil composition comprising an oil of lubricating viscosity and from 0.2 to 10 percent by weight of a product as defined in claim 5.

14. A lubricating oil concentrate comprising from about 90 to 10 weight percent of an oil of lubricating viscosity and from about 10 to 90 weight percent of a product as defined in claim 1.

15. A lubricating oil concentrate comprising from about 90 to 10 weight percent of an oil of lubricating viscosity and from about 10 to 90 weight percent of a product as defined in claim 2.

16. A lubricating oil concentrate comprising from about 90 to 10 weight percent of an oil of lubricating viscosity and from about 10 to 90 weight percent of a product as defined in claim 3.

17. A lubricating oil concentrate comprising from about 90 to 10 weight percent of an oil of lubricating viscosity and from about 10 to 90 weight percent of a product as defined in claim 4.

18. A lubricating oil concentrate comprising from about 90 to 10 weight percent of an oil of lubricating viscosity and from about 10 to 90 weight percent of a product as defined in claim 5.

19. A process for the preparation of modified amino-decorated hydrocarbon polymers which comprises contacting at a temperature sufficient to cause reaction an amino-decorated hydrocarbon polymer having at least one primary or secondary amine group with a cyclic carbonate and wherein the molar charge of cyclic car-



wherein R<sub>1</sub>, R<sub>2</sub>, R<sub>3</sub>, R<sub>4</sub>, R<sub>5</sub> and R<sub>6</sub> are independently selected from hydrogen or alkyl of 1 to 2 carbon atoms; and n is an integer from 0 to 1.

3. A product prepared as in the process of claim 2 wherein the cyclic carbonate is



4. A product prepared as in the process of claim 3 wherein n is zero; R<sub>1</sub>, R<sub>2</sub> and R<sub>5</sub> are hydrogen; and R<sub>6</sub> is hydrogen or methyl.

5. A product prepared as in the process of claim 4 wherein R<sub>6</sub> is hydrogen.

6. A product prepared as in the process of claim 1 wherein the reaction is conducted at from 0° to 250° C.

7. A product prepared as in the process of claim 1 wherein the molar charge of the cyclic carbonate to the basic nitrogens of the amino-decorated hydrocarbon polymer viscosity index is from about 0.5:1 to about 5:1.

8. A product prepared as in the process of claim 7 wherein the molar charge of the cyclic carbonate to the basic nitrogens of the amino-decorated hydrocarbon polymer is from about 1:1 to about 3:1.

9. A lubricating oil composition comprising an oil of lubricating viscosity and from 0.2 to 10 percent by weight of a product as defined in claim 1.

10. A lubricating oil composition comprising an oil of lubricating viscosity and from 0.2 to 10 percent by weight of a product as defined in claim 2.

11. A lubricating oil composition comprising an oil of lubricating viscosity and from 0.2 to 10 percent by weight of a product as defined in claim 3.

12. A lubricating oil composition comprising an oil of lubricating viscosity and from 0.2 to 10 percent by weight of a product as defined in claim 4.

13. A lubricating oil composition comprising an oil of lubricating viscosity and from 0.2 to 10 percent by weight of a product as defined in claim 5.

14. A lubricating oil concentrate comprising from about 90 to 10 weight percent of an oil of lubricating viscosity and from about 10 to 90 weight percent of a product as defined in claim 1.

15. A lubricating oil concentrate comprising from about 90 to 10 weight percent of an oil of lubricating viscosity and from about 10 to 90 weight percent of a product as defined in claim 2.

16. A lubricating oil concentrate comprising from about 90 to 10 weight percent of an oil of lubricating viscosity and from about 10 to 90 weight percent of a product as defined in claim 3.

17. A lubricating oil concentrate comprising from about 90 to 10 weight percent of an oil of lubricating viscosity and from about 10 to 90 weight percent of a product as defined in claim 4.

18. A lubricating oil concentrate comprising from about 90 to 10 weight percent of an oil of lubricating viscosity and from about 10 to 90 weight percent of a product as defined in claim 5.

19. A process for the preparation of modified amino-decorated hydrocarbon polymers which comprises contacting at a temperature sufficient to cause reaction an amino-decorated hydrocarbon polymer having at least one primary or secondary amine group with a cyclic carbonate and wherein the molar charge of cyclic car-

bonate to the basic nitrogens of the amino-decorated hydrocarbon polymer is from about 0.2:1 to about 10:1.

20. The process of claim 19 wherein the cyclic carbonate is selected from the group consisting of



10

15 wherein  $R_1$ ,  $R_2$ ,  $R_3$ ,  $R_4$ ,  $R_5$  and  $R_6$  are independently selected from hydrogen or alkyl of 1 to 2 carbon atoms; and  $n$  is an integer from 0 to 1.

-continued



20

25

30

35

40

45

50

55

60

65